

1

3,009,796

## GAS-PRODUCING COMPOSITIONS OF SMOKE-LESS POWDER AND METAL COMPOUND INHIBITORS

Ralph F. Preckel, Frostburg, Md., assignor, by mesne assignments, to the United States of America as represented by the Secretary of the Navy  
No Drawing. Filed Mar. 8, 1951, Ser. No. 214,629  
1 Claim. (Cl. 52—5)

The present application is a continuation-in-part of my copending application entitled, "Gas-Producing Charge," Serial No. 102,427, filed June 30, 1949, now abandoned, and as in the case of said previously filed application, the present invention relates to smokeless powders and more particularly to smokeless powders having ballistic characteristics peculiarly desirable for application in jet actuated devices.

It is well known that there is a definite and direct relationship between the pressure at which a smokeless powder propellant burns and its burning rate. This relationship may be mathematically expressed as  $r=cp^n$ , or as  $\log r=n \log P + \log c$ , where  $r$  is the burning rate,  $P$  is the pressure at which the burning rate is measured, and  $c$  and  $n$  are constants characteristic of a given propellant. Thus, when a plot of  $\log r$  against  $\log P$  is made for the conventional propellant, a straight line of slope  $n$  is obtained showing an increase in burning rate for each increase in pressure. Such a relationship is not disadvantageous in the conventional propellant, and in fact is used to advantage in progressive powders where it is highly desirable to generate increased pressures after the projectile or shot charge has begun to move along the barrel. However, this relationship presents a serious problem in formulation of propellants for jet-actuated devices, since once the desired operating pressure is reached, totally different considerations obtain.

It is highly desirable, once the operating pressure of a jet-actuated device is reached, that the pressure generated by the burning propellant be maintained as nearly constant as possible. Accordingly, if this result is to be attained, the slope  $n$  of the line representing the pressure-burning rate relationship of the particular propellant should preferably approach zero in the zone of useful rocket pressure. In the prior art rocket powders, in all of which the slope  $n$  has a value of 0.7 or over, any fracturing or slivering of the propellant charge leads to a pressure build-up because of an increase in linear burning rate resulting from the increase in pressure due to the increase in burning surface. The higher the  $n$  value of the particular powders, the higher will be the pressure rise encountered. Therefore, the results of such a fracturing or slivering vary from a highly undesirable thrust fluctuation, with consequent aberration in ballistics, to actual failure of the jet device if, as with a propellant of high  $n$  value, the pressure build-up is excessive. Even unusual roughness of the charge causes serious changes in burning pressure and burning rate in the presently available rocket propellants, with the result that errors of 1% in the nozzle diameter have been found to build up to an aberration of 5% or more in ballistics. Consequently, with the propellants now available, there is very little allowable tolerance in manufacture of charges and nozzles for jet devices. A propellant having a very low  $n$  value within the range of useful rocket pressures, however, would allow for considerable tolerances without appreciable deviation from the specified ballistics, and accordingly any decrease in  $n$  value would accordingly enhance the value of a particular propellant.

A second serious problem confronting producers of propellants for jet-actuated devices is the diminution of the temperature coefficient of equilibrium pressure at the

2

desired operating pressure or pressure range. The temperature coefficient of equilibrium pressure is a measure of the pressure variation to be expected from a given propellant on account of temperature variation alone.

It is obtained by firing identical samples of propellant under identical conditions except for changes in temperature and pressure. The coefficient may be expressed as

$$\frac{\Delta P}{\bar{P} \Delta t}$$

where  $\Delta P$  is the experimentally determined difference in pressure under conditions of equilibrium burning due to the temperature change  $\Delta t$ , and  $\bar{P}$  is the mean of the low-temperature and high-temperature pressures.

The advantage of having a low-temperature coefficient of equilibrium pressure is obvious. If the coefficient is low, the jet-actuated device may be designed for an unusually low range of service pressure over the wide temperature range ordinarily specified for such devices in field use. Since existing propellants generally have temperature coefficients of equilibrium pressure of about 0.8%/° C. or more, service pressure may change by 100% or more in going from the lowest expected temperature (about -55° C.) to the highest expected temperature (about 75° C.). It is therefore highly desirable to lower the temperature coefficient of equilibrium pressure below that of existing rocket propellants and thereby hold variations in service pressure due to temperature changes to a minimum. If the coefficient could be lowered from 0.8%/° C. to 0.4%/° C. or less, service pressure variation would be diminished by at least one half, and similarly any lowering of this temperature coefficient would correspondingly enhance the value of the propellant.

As a result of the advantages set forth above for a propellant having a low  $n$  value and/or a low temperature coefficient of equilibrium pressure, either or both of these two ballistic characteristics would allow for important economies in the inert weight of jet-actuated devices. This is clearly seen if the equation is examined which relates the ratio between the mass of propellant ( $m$ ) and the mass of the jet device without propellant ( $M$ ), the gas velocity of the burning propellant ( $V$ ), and the highest theoretically obtainable velocity of the jet device ( $V_{max.}$ ) as follows:

$$V_{max.} = 2.303 V \log_{10} \left( 1 + \frac{m}{M} \right)$$

With propellants now available, the highest ratio of  $m/M$  has been about 1, where mass of propellant and mass of jet device are about equal. If it is possible, by use of a new propellant which does not build up excessive pressures, to decrease  $M$  by 10% and increase the amount of propellant to give the same total initial weight,  $V_{max.}$  would be increased by a factor

$$\frac{\log_{10} \left( 1 + \frac{1.1}{0.9} \right)}{\log_{10} \left( 1 + \frac{1}{1} \right)}$$

or about 1.15. This would be a 15% improvement.

Therefore, an object of the present invention is the production of propellants for jet-actuated devices which are characterized by low burning rate-pressure relationships throughout a wide pressure region within the range of useful rocket pressures.

A further object of this invention is the production of propellants for jet-actuated devices which are characterized by low temperature coefficients of equilibrium pressure, thus minimizing variations in service pressure due to temperature.

The previously mentioned copending application is directed to smokeless powder propellant explosives which

have incorporated therein at least one material selected from the group consisting of lead and compounds of lead, and which have heats of explosion of not more than about 900 calories per gram. As there described, the addition of these materials to said propellants causes a substantial reduction in the  $n$  value and the temperature coefficient of equilibrium pressure over that obtained in the absence of said additives. In accordance with the present invention, it has been found that similar effects, lowering of  $n$  value and in some cases lowering of the temperature coefficient of equilibrium pressure, are had upon the same propellants and types of propellants described in said previous application by uniformly incorporating therein minor amounts of many other metals and compounds of metals, as more specifically set out hereinbelow, provided these compositions of propellant and modifier have heats of explosion of not more than about 900 calories per gram. As pointed out in detail in the earlier mentioned application with specific reference to the lead and compounds of lead modifiers, the smokeless powders to which these ballistic modifiers are added may be either single or multiple base powders. If the smokeless powder to which one or more of the ballistic modifiers is added is a single-base powder, it should preferably comprise from 85 to 95% nitrocellulose and from 5 to 15% plasticizer. If the propellant used in a multiple-base formula, it should preferably comprise from 40 to 85% nitrocellulose, from 10 to 35% of an explosive liquid ester, and from 5 to 30% of a substantially nonvolatile nonexplosive plasticizer. In any formulation, however, it is critical that the heat of explosion of the additive system be not greater than about 900 calories per gram. For, as shown in said previous application, where formulations have heats of explosion in excess of said amount, the additive ballistic modifiers lose a considerable amount of their effectiveness in suppressing the  $n$  value and the temperature coefficient of equilibrium pressure in cases where the latter suppression is effected. As further pointed out in said application, the heats of explosion of various formulations can be readily calculated by one skilled in the art to determine whether the formulations are suitable for the purposes of the present invention. Smokeless powder propellants prepared in accordance with this invention, i.e. containing minor amounts of the modifiers listed hereinbelow and having heats of explosion which do not exceed about 900 calories per gram, are characterized by a pressure-burning rate relationship having a substantially lower  $n$  value and in some cases a substantially lower temperature coefficient of equilibrium pressure than is possessed by the propellant in the absence of the modifiers. It has been found that up to 10% of the various operable additives may be employed without adversely affecting the ballistics of the gas-producing compositions of the invention, however, it is preferred to employ only sufficient amounts of additives to effect the desired modification in ballistics. In most cases it has been found that 2% of the various additives, based on the weight of the smokeless powder employed, is ample.

Having now generally described the invention, the following table presents a plurality of examples of ballistic modifiers which when employed in accordance with the present invention provide substantial decreases in the  $n$  value of smokeless powder propellant explosives, and, as will be noted, in some instances also effect a substantial reduction in the propellant's temperature coefficient of equilibrium pressure. This table indicates the heat of explosion, lowest  $n$ , pressure region of lowest  $n$ , and temperature coefficient of pressure in region of lowest  $n$  for a standard rocket propellant composition having the following formulation.

|                           | Percent |
|---------------------------|---------|
| Nitrocellulose (13.15% N) | 58.5    |
| Nitroglycerin             | 22.5    |
| Triacetin                 | 8.5     |
| Ethyl centralite          | 8.0     |
| Dinitrotoluene            | 2.5     |

when indicated modifiers are added thereto in amounts stated.

| Ex. | Modifier                                       |               | Heat of explosion cal./g. | Lowest $n$ | Pressure region of lowest $n$ p.s.i. | Temp. coef. of pressure in region of lowest $n$ percent/ $^{\circ}$ C. |
|-----|------------------------------------------------|---------------|---------------------------|------------|--------------------------------------|------------------------------------------------------------------------|
|     | Type                                           | Amt., percent |                           |            |                                      |                                                                        |
| 10  | No addition                                    |               | 700                       | 0.7        |                                      | 0.8                                                                    |
| 2   | Ag. pwd.                                       | 0.5           | 700                       | 0.3        | 1,400-3,000                          | 0.3                                                                    |
| 3   | Ag. pwd.                                       | 2.0           | 685                       | 0.2        | 1,500-3,300                          | 0.3                                                                    |
| 4   | Ag. pwd.                                       | 4.0           | 675                       | 0.2        | 1,400-3,600                          | 0.2                                                                    |
| 5   | Ag <sub>2</sub> O                              | 1.0           | 695                       | 0.3        | 1,000-2,000                          | 0.3                                                                    |
| 6   | Sb <sub>2</sub> O <sub>3</sub>                 | 1.0           | 695                       | 0.2        | 1,300-1,800                          | 0.2                                                                    |
| 7   | Sb pwd.                                        | 1.0           | 695                       | 0.3        | 2,000-2,400                          | 0.4                                                                    |
| 8   | MnCO <sub>3</sub>                              | 1.0           | 695                       | 0.2        | 1,300-2,400                          | 0.5                                                                    |
| 9   | Pd pwd.                                        | 0.5           | 700                       | 0.3        | 1,000-2,350                          | 0.3                                                                    |
| 10  | Cu <sub>2</sub> O                              | 1.0           | 695                       | 0.3        | 1,000-2,500                          | 0.6                                                                    |
| 11  | Cu <sub>2</sub> O                              | 2.0           | 685                       | 0.2        | 1,300-2,000                          | 0.4                                                                    |
| 12  | CuCO <sub>3</sub>                              | 1.0           | 695                       | 0.4        | 1,300-2,000                          | 0.7                                                                    |
| 13  | Cu(OH) <sub>2</sub> (basic carbonate).         |               |                           |            |                                      |                                                                        |
| 14  | CdO                                            | 1.0           | 695                       | 0.3        | 1,500-2,650                          | 0.4                                                                    |
| 15  | CdCO <sub>3</sub>                              | 1.0           | 695                       | 0.6        | 900-2,000                            | 1.2                                                                    |
| 16  | Cd                                             | 1.0           | 695                       | 0.5        | 1,300-2,000                          | 0.7                                                                    |
| 17  | Bi pwd.                                        | 1.0           | 695                       | 0.4        | 1,500-2,400                          | 0.6                                                                    |
| 18  | Bi <sub>2</sub> O <sub>3</sub>                 | 1.0           | 695                       | 0.4        | 1,300-2,200                          | 0.3                                                                    |
| 19  | (BiO) <sub>2</sub> CO <sub>3</sub>             | 1.0           | 695                       | 0.4        | 1,500-2,250                          | 0.9                                                                    |
| 20  | xH <sub>2</sub> O (subcarbonate).              |               |                           |            |                                      |                                                                        |
| 21  | Amorphous B.                                   | 1.0           | 695                       | 0.4        | 2,500-4,000                          | 0.4                                                                    |
| 22  | Mo pwd.                                        | 1.0           | 695                       | 0.4        | 1,000-2,600                          | 0.4                                                                    |
| 23  | U <sub>3</sub> O <sub>8</sub> (uranium oxide). | 1.0           | 695                       | 0.4        | 620-1,350                            | 0.3                                                                    |
| 24  | BaCO <sub>3</sub>                              | 1.0           | 695                       | 0.4        | 1,100-2,000                          | 0.4                                                                    |
| 25  | V <sub>2</sub> O <sub>5</sub>                  | 1.0           | 695                       | 0.4        | 1,400-1,900                          | 0.4                                                                    |
| 26  | ThO <sub>2</sub>                               | 1.0           | 695                       | 0.5        | 1,200-2,700                          | 0.5                                                                    |
| 27  | Ta <sub>2</sub> O <sub>5</sub>                 | 1.0           | 695                       | 0.5        | 1,100-1,900                          | 0.4                                                                    |
| 28  | Cr pwd.                                        | 1.0           | 695                       | 0.5        | 1,300-2,750                          | 0.4                                                                    |
| 29  | Co <sub>2</sub> O <sub>3</sub>                 | 1.0           | 695                       | 0.5        | 100-500                              | 1.2                                                                    |
| 30  | Co pwd.                                        | 1.0           | 695                       | 0.6        | 1,500-2,500                          | 0.7                                                                    |
| 31  | Se pwd.                                        | 1.0           | 695                       | 0.5        | 1,250-2,200                          | 0.4                                                                    |
| 32  | CaCO <sub>3</sub>                              | 1.0           | 695                       | 0.5        | 1,600-3,000                          | 0.5                                                                    |
| 33  | Au pwd.                                        | 0.5           | 700                       | 0.5        | 1,350-3,100                          | 0.6                                                                    |
| 34  | TiO <sub>2</sub>                               | 1.0           | 695                       | 0.5        | 1,000-4,000                          | 1.4                                                                    |
| 35  | S pwd.                                         | 1.0           | 695                       | 0.5        | 300-800                              | 1.6                                                                    |
| 36  | Dibutyltin diacetate.                          | 1.0           | 680                       | 0.5        | 200-600                              | 0.6                                                                    |
| 37  | Tetraphenyl tin.                               | 0.5           | 690                       | 0.6        | 1,250-2,150                          | 0.6                                                                    |
| 38  | SnO                                            | 1.0           | 695                       | 0.6        | 300-840                              | 1.6                                                                    |
| 39  | Sn pwd.                                        | 1.0           | 695                       | 0.6        | 1,100-3,000                          | 1.1                                                                    |
| 40  | W pwd.                                         | 1.0           | 695                       | 0.6        | 1,300-4,000                          | 0.4                                                                    |
| 41  | NiO                                            | 1.0           | 695                       | 0.6        | 300-4,000                            | 0.7                                                                    |
| 42  | KI                                             | 1.0           | 695                       | 0.6        | 300-3,000                            | 0.7                                                                    |
|     | CsNO <sub>3</sub>                              | 1.0           | 695                       | 0.6        | 300-4,000                            | 0.9                                                                    |

From the examples given in the foregoing table, it is apparent that although all of the ballistic modifiers there disclosed are operable in lowering  $n$  value, a wide range of variations in effect on  $n$  value and on temperature coefficient of pressure is had between the several types of modifiers, and further such variations are found to occur as a result of variations in the percentage amount of a particular modifier employed. These facts provide for considerable flexibility in employing the teachings of the present invention, enabling a wide choice of modifiers and amounts thereof based on economic considerations as well as the ballistics desired for a particular application of the invention. By reference to the foregoing table, one skilled in the art can readily determine the nature and amount of modifier appropriate for accomplishing the desired ballistic modifications. Many examples of propellant powder formulations found to respond as indicated to additions of small percentages of said modifiers have been disclosed in my copending application above-identified, and furthermore said application clearly discloses the general principles and criteria for determining whether or not a particular propellant powder will respond in the manner indicated in the foregoing description of the present invention.

The foregoing specific examples of modifiers and amounts of modifiers employed, and the particular propellant powder formulation indicated are presented merely by way of example, to clearly indicate the nature and significance of the present invention. Modifications of these details will be apparent to those skilled in the

art, and such modifications as are within the spirit and scope of the present invention as defined by the appended claim are within the contemplation of the present patent.

What is claimed is:

The method of diminishing the  $n$  value and temperature coefficient of equilibrium pressure of a double base rocket propellant in a pressure region suitable for operation of a rocket device, said propellant comprising 40-85% nitrocellulose and 10-35% nitroglycerine and having a heat of explosion not to exceed 900 calories per gram, comprising uniformly dispersing throughout said composition a ballistic modifier selected from the group consisting of silver and silver oxide in quantities adequate to obtain the desired reduction in said  $n$  value and temperature coefficient but not to exceed 10% by weight of said propellant, wherein the  $n$  value of said propellant is the slope of the plot of the log of the burning rate ( $r$ ) against the log of the pressure ( $p$ ) at which the burning

rate is measured, and the temperature coefficient is equal to  $\Delta P/\bar{p}\Delta t$  wherein  $\Delta P$  is the difference in pressures due to the temperatures change  $\Delta t$  and  $\bar{p}$  is the mean of the pressures.

References Cited in the file of this patent

UNITED STATES PATENTS

|    |           |              |                |
|----|-----------|--------------|----------------|
| 10 | 1,336,463 | Henning      | Apr. 13, 1920  |
|    | 1,357,865 | Henning      | Nov. 2, 1920   |
|    | 1,943,421 | Burns et al. | Jan. 16, 1934  |
|    | 1,963,116 | Burns et al. | June 19, 1934  |
|    | 2,038,700 | Woodbridge   | Apr. 28, 1936  |
| 15 | 2,131,352 | Marsh        | Sept. 27, 1938 |
|    | 2,344,840 | Watt et al.  | Mar. 21, 1944  |

FOREIGN PATENTS

|         |               |               |
|---------|---------------|---------------|
| 621,685 | Great Britain | Apr. 14, 1949 |
|---------|---------------|---------------|